# EUROPEAN PATENT SPECIFICATION

(11) **EP 2 984 198 B1**
(45) Date of publication and mention of the grant of the patent: **23.06.2021**
(21) Application number: 14716760.5
(22) Date of filing: 09.04.2014
(51) Int. Cl.: C22C 38/00, C21D 1/00

(54) **PRODUCT FORMED BY HOT FORMING OF METALLIC COATED STEEL SHEET, METHOD TO FORM THE PRODUCT, AND STEEL STRIP**
AUS WARMUMFORMUNG VON METALLISCHEM BESCHICHTETEM STAHLBLECH HERGESTELLTES PRODUKT, VERFAHREN ZUR HERSTELLUNG DES PRODUKTS, UND STAHLBLECH
PRODUIT FORMÉ PAR FORMAGE À CHAUD DE TÔLE D'ACIER À REVÊTEMENT MÉTALLIQUE, PROCÉDÉ POUR FORMER LE PRODUIT ET BANDE D'ACIER

(30) Priority: 10.04.2013 EP 13001845
(43) Date of publication of application: 17.02.2016
(73) Proprietor: Tata Steel IJmuiden B.V., NL-1951 JZ VELSEN-NOORD (NL)
(72) Inventor: CHEN, Shangping, NL-1951 JZ Velsen-Noord (NL); HENSEN, Guido Cornelis, NL-1951 JZ Velsen-Noord (NL)
(74) Representative: Group Intellectual Property Services
(86) International application number: PCT/EP2014/000951
(87) International publication number: WO 2014/166630

(56) References cited:
- EP-A1- 2 053 139
- EP-A1- 2 220 259
- WO-A1-2010/069588
- WO-A1-2014/037627
- DE-B3-102009 044 861
- DE-U1-202012 000 616
- GB-A- 2 527 384
- JP-A- 2001 064 751
- JP-A- 2011 208 164
- US-A1- 2012 006 451
- KARBASIAN H ET AL: "A review on hot stamping", JOURNAL OF MATERIALS PROCESSING TECHNOLOGY, ELSEVIER, NL, vol. 210, no. 15, 19 November 2010 (2010-11-19), pages 2103-2118, XP027378020, ISSN: 0924-0136 [retrieved on 2010-08-06]

## Description

The invention relates to a product formed by hot forming of a metallic coated steel sheet, wherein the formed product has a substrate layer of hot formed steel, a metal affected zone and a diffusion coating layer on the substrate layer, and optionally a metal oxide layer on the diffusion coating layer. The invention also relates to a method for producing such a product, and to a steel strip for use in the method.

Products formed by hot forming are well known in the art. Such products have the advantage that, starting from a blank having a low strength, products with high mechanical properties (such as a high tensile strength) can be produced, which products do not show spring-back. However, during production the steel oxidizes. For this reason, in recent years metallic coated blanks are used to produce hot formed products. As a coating aluminium or an aluminium alloy, or zinc or a zinc alloy can be used. The steel substrate usually is a so-called boron steel.

It has been found that the use of such coatings has the disadvantage that the formability of the steel sheet is hampered, and more specific, the bendability of the coated steel sheets after hot forming is reduced; and that especially for zinc (alloy) coated steel sheets micro-cracks are formed during the hot and/or cold forming process. Bendability is the property of being easily bent without breaking, measured by bending angle at maximum force in a three-point bending test. Higher bendability can have a positive influence on the crash behaviour. Micro-cracks are usually present in the coating, but due to high stresses in the product micro-cracks can also be introduced in the surface of the substrate steel. These micro-cracks occur in particular in areas that are formed with a high degree of deformation.

DE 10 2009 044 861 B3 discloses a method for manufacturing a high ductile steel, wherein the step of annealing is executed at a temperature of 600 - 1100° for a period of 10 - 360 seconds to provide the product with a 10 - 200 µm thick ductile layer, having a ductility which is higher than the ductility of the core of the product. The product may be provided with a metallic - anorganic coating.

WO2014/037627 discloses a pre-coated laminated sheet for manufacturing press hardened parts, which has a steel substrate and a metal pre-coating on the steel substrate, wherein there is a decarbonated zone on the surface of the main faces of the steel substrate. The laminated sheet is hot formed into a product.

It is an object of the present invention to provide a metallic coated hot formed product having an improved formability.

It is another object of the present invention to provide a zinc coated hot formed product having less and/or smaller micro-cracks.

It is also an object of the invention to provide a method for producing a metallic coated hot product, having improved bendability and/or less/smaller micro-cracks.

Furthermore, it is an object of the invention to provide a hot formable steel strip that can be used for forming such products.

According to a first aspect of the invention a product is provided formed by hot forming of a metallic coated steel sheet, wherein the formed product has a substrate of hot formed steel, a metal affected zone and a diffusion coating layer on the substrate, and optionally a metal oxide layer on the diffusion coating layer, wherein a low carbon zone is present between the substrate layer and the metal affected zone, and the product is formed by providing a decarburized zone in the substrate steel before coating to reduce the depth of the metal affected zone and by controlling the thickness of the decarburized zone in the steel sheet such that it is larger than the sum of the thickness of the diffusion coating layer and the thickness of the metal affected zone to ensure the formation of the low carbon layer.

The metal affected zone is the zone directly under the diffusion layer, where the metal of the coating has penetrated into the substrate steel in a small amount under industrial production conditions. The inventors have realized that the small amount of the coating element such as Zn will segregate at the original austenite grain boundaries in the metal affected zone, which is the main cause for the formation of the microcracks during forming, and therefore, the depth of the metal affected zone should be minimized. The inventors have found that the presence of a low carbon zone in the substrate steel before coating can reduce the depth of the metal affected zone between the substrate and the diffusion coating layer during production process. In the one hand, the inventors assume that the low carbon layer will help to minimize liquid zinc penetration in the substrate and/or solid zinc diffusion into the substrate. On the other hand, the inventors assume that the low carbon zone forms a ductile layer between the substrate and the metal affected zone during heating for hot press forming, which will dissipate tensions during the hot forming and/or cold forming (after hot forming), resulting in an improved formability. Therefore, the tendency to form micro-cracks during hot forming is reduced. The bendability of the coated sheets is also increased.

Preferably the metal of the metallic coated steel sheet is zinc or a zinc alloy, or aluminium or an aluminium alloy. These are nowadays the coatings that provide the best corrosion protection of the hot formed products.

According to a preferred embodiment the low carbon zone has a carbon content of at most 0.01 weight% C. With a carbon content of at most 0.01 weight%, the low carbon zone has the required ductility.

According to a preferred embodiment the metal affected zone has a thickness less than 10 µm, preferably less than 5 µm. The metal affected zone should be as small as possible. By providing a proper decarburized zone in the steel sheet before coating, the thickness of the metal affected zone is reduced; and a low carbon layer is eventually formed between the substrate and the metal affected zone during coating and the following production processes. Depending on the coating types, the thickness of the coating layer and the hot press forming temperature, the thickness of the diffusion coating layer and the thickness of the metal affected zone vary.

Preferably, the low carbon layer has a thickness of up to 30 µm, preferably between 5 and 30 µm, more preferably between 5 and 20 µm, most preferably between 5 and 10 µm. The thickness of the low carbon layer should be not so large to influence the mechanical properties of the hot formed product.

Preferably, the metal of the metallic coated steel sheet is galvannealed zinc, or a zinc alloy containing (in weight %) 0.1- 6 Al, 0 - 6 Mg and optionally at most 0.2 weight% of Pb, Sb, Ti, Ca, Mn, Sn, La, Ce, Cr, Ni, Zr and/or Bi each, the remainder being zinc and unavoidable impurities, and preferably 0.1 - 3 Al, 0 - 3 Mg and at most 0.2 weight% of Pb, Sb, Ti, Ca, Mn, Sn, La, Ce, Cr, Ni, Zr and/or Bi each, the remainder being zinc and unavoidable impurities, or wherein the metal of the metallic coated steel sheet is a zinc-nickel alloy containing (in weight%) 0.2 - 7 Ni, the remainder being zinc and unavoidable impurities, or wherein the metal of the metallic coated steel sheet is an aluminium alloy containing (in weight%) 6 - 12 Al and/or 1 - 5 Fe, the remainder being aluminium and unavoidable impurities. These coatings can provide a good corrosion protection during and after the hot forming process. Usually at most 0.1 weight% of Pb, Sb, Ti, Ca, Mn, Sn, La, Ce, Cr, Ni, Zr and/or Bi each is present in the zinc alloy, or even at most 0.02 weight%. Preferably in the zinc alloy 1.0 - 2.5 Al and 1.0 - 2.5 Mg is present, more preferably 1.5 - 1.8 Al and 1.5 - 1.8 Mg.

The substrate layer of hot formed steel has been made from a steel having the following composition in weight %:
C: 0.10 - 0.5, preferably 0.15 - 0.4
Mn: 0.5 - 3.0, preferably 1.0 - 2.5
Si: 0.1 - 0.5, preferably 0.1 - 0.4
Cr: up to 1.0, preferably up to 0.8
Ti: up to 0.2, preferably up to 0.1
Al: up to 0.2, preferably up to 0.1
P: up to 0.1, preferably up to 0.08
S: up to 0.05, preferably up to 0.04
B: 0.0005 - 0.08, preferably 0.0005 - 0.04
optionally Nb up to 2, preferably up to 0.1
optionally V up to 2, preferably up to 0.1
optionally W up to 3, preferably up to 0.1
the remainder being iron and unavoidable impurities.
Steel having this composition is suitable for hot forming.

According to a second aspect of the invention a method for producing a metallic coated hot formed product is provided, the method comprising the following steps:
- providing a strip of hot formable steel having a decarburized zone with a controlled depth at both sides of the strip of steel;
- providing a metallic coating on the decarburized steel strip;
- cutting a blank from the coated strip of metal;
- hot forming the coated blank or preformed part into a metallic coated hot formed product.

According to the invention a decarburized zone is formed at both sides of the steel strip before the steel strip is coated with a metallic coating, also at both sides of the steel strip. The depth of the decarburized zone has to be such that after the hot forming of the product, a low carbon zone is still present between the steel substrate and the metal affected zone.

Preferably the hot forming is performed by either heating the blank, hot pressing the blank into a formed product, and quenching the formed product, or cold pressing the blank into a preformed product, heating the preformed product, hot pressing the preformed product into a formed product, and quenching the formed product. These two hot forming methods are usually called the direct method and the indirect method. After quenching the hot formed product must be trimmed, and optionally part or all of the metal oxides are removed.

According to a preferred method the decarburized zone has been provided to a depth of 20 to 50 µm, preferably a depth of 35 to 45 µm, more preferably a depth of 30 to 40 µm. During the subsequent method steps the decarburization zone in the hot formed product will be reduced, also depending on the thickness of the metallic coating and the heating before the hot forming step. By providing a proper decarburized zone in the steel sheet before coating, the thickness of the metal affected zone is reduced; and a low carbon layer is eventually formed between the substrate and the metal affected zone during coating and the following production processes. Depending on the coating types, the thickness of the coating layer and the hot press forming temperature, the thickness of the diffusion coating layer and the thickness of the metal affected zone vary. Therefore, the thickness of the decarburized zone in the steel sheet should be controlled such that it is larger than the sum of the thickness of the diffusion coating layer and the thickness of the metal affected zone to ensure the formation of the low carbon layer.

According to a first preferred embodiment of the method the decarburized zone is provided in an annealing line by applying a dew point higher than - 20 °C in an (N2 + H2) atmosphere. In this way, during the continuous annealing a decarburized zone is formed on both sides of the steel strip.

Preferably, annealing is performed at 740 to 860 °C for 30 - 240 seconds in a N2 + 2-5% H2 atmosphere with a dew point in the range from -15 °C to 5 °C. It has been found that in this way a proper decarburized zone is formed having the required depth.

According to a second preferred embodiment of the method the decarburized zone is provided by cooling a hot rolled strip of hot formable steel from a finishing rolling temperature between the Ac1 and the Ac3 temperature to the coiling temperature between 450 °C and 750 °C. During the cooling of the strip on the run-out table the decarburized zone is formed.

Preferably, the metallic coating on the steel strip is provided as a zinc or zinc alloy, or aluminium or aluminium alloy coating, more preferably by using hot-dip coating. These coatings are the most used for hot forming.

The strip of hot formable steel used has the following composition in weight %:
C: 0.10 - 0.5, preferably 0.15 - 0.4
Mn: 0.5 - 3.0, preferably 1.0 - 2.5
Si: 0.1 - 0.5, preferably 0.1 - 0.4
Cr: up to 1.0, preferably up to 0.8
Ti: up to 0.2, preferably up to 0.1
Al: up to 0.2, preferably up to 0.1
P: up to 0.1, preferably up to 0.08
S: up to 0.05, preferably up to 0.04
B: 0.0005 - 0.08, preferably 0.0005 - 0.04
optionally Nb up to 2, preferably up to 0.1
optionally V up to 2, preferably up to 0.1
optionally W up to 3, preferably up to 0.1
the remainder being iron and unavoidable impurities.
Steel with such a composition is suitable for hot forming.

A hot formable steel strip for use in the method according to the second aspect of the invention is provided, the steel strip having a composition in weight % of:
C: 0.10 - 0.5, preferably 0.15 - 0.4
Mn: 0.5 - 3.0, preferably 1.0 - 2.5
Si: 0.1 - 0.5, preferably 0.1 - 0.4
Cr: up to 1.0, preferably up to 0.8
Ti: up to 0.2, preferably up to 0.1
Al: up to 0.2, preferably up to 0.1
P: up to 0.1, preferably up to 0.08
S: up to 0.05, preferably up to 0.04
B: 0.0005 - 0.08, preferably 0.0005 - 0.04
optionally Nb up to 2, preferably up to 0.1
optionally V up to 2, preferably up to 0.1
optionally W up to 3, preferably up to 0.1
the remainder being iron and unavoidable impurities,
wherein the strip at both sides has a decarburized zone to a depth of 20 to 50 µm, preferably a depth of 30 to 40 µm.
This steel strip, at both sided provided with a decarburized zone, is suitable for use in the method for producing a hot formed product according to the invention, which has a better bendability and a better resistance against micro-cracks .

The invention will be elucidated using the accompanying figures, also providing an example.

Figure 1 gives a schematic description of the process steps according to the invention.

Figure 2 shows the bending angle of the coated steel according to the invention in comparison with the prior art.

Figure 1 shows the sequence of steps in the process from start to finished product schematically. Step A shows the substrate 1 of the steel strip that is the starting point of the process. Step B shows that in the top layer of the substrate a decarburization zone 2 has been formed. Though the decarburization zone is part of the steel strip, for clarity the decarburization is described as a layer on top of the substrate. Though not shown, usually on both sides of the substrate a decarburization zone is formed. The decarburization zone can for instance be formed during continuous annealing, as described hereunder. In step C a coating layer 3 has been applied on the substrate with the decarburization layer. The coating layer can for instance be applied using a hot dip coating process. Step D shows the endpoint of the process, after the hot forming of a blank with the structure as seen in step C. On top, an oxide layer 6 of the coating material is formed. Under the oxide layer, a diffused layer 5 is formed, where the steel from the decarburization zone has diffused with the coating material. Directly below the diffused layer a metal affected zone 4 is formed, where the decarburized zone has been partially consumed by the diffusion coating layer. Between the substrate and the metal affected zone is shown what remains of the decarburization zone in the form of a low carbon zone 2. These layers are usually already formed during the heating of the blank before the hot press forming in a hot forming press.

It will be clear that the thickness of the oxide layer, the diffused layer and the metal affected zone will depend on a number of variables. Clearly the type of metallic coating is such a variable, and also the thickness of this coating layer, but probably also the heating time of the blank before the hot press forming, and the heating temperature of the blank.

However, the inventors have found that when a GA 130 coating is used and the blank is heated in a preheated furnace of 900° C during approximately 5 minutes, a decarburization zone with a depth of 30 to 40 µm can be used (as shown in step B of Figure 1), so as to obtain a low carbon zone in the range of 5 to 10 µm in the hot formed product (as shown in step D of Figure 1). With some routine experiments the required decarburization depth on the substrate of the steel strip can be found for a different coating, another coating thickness, and, if needed, another furnace temperature and heating time.

An example for the production of a decarburization zone is as follows. A cold rolled strip of 22MnB5 steel having a thickness of 1.5 mm is continuously annealed at a temperature of approximately 800° C during about 120 seconds in a N2 + 2% H2 atmosphere with a dew point of -5° C. In this way, a decarburization zone with a depth of approximately 35 µm is obtained.

The steel strip is then cooled to about 460° C at a rate of about 10° C/sec, held for about 2 seconds at 460° C, and then hot-dipped in a Zinc bath of 460 °C. The zinc bath contains 0.19 wt% aluminium and 0.011 wt% iron. After the hot dip coating, the coated steel strip is wiped with nitrogen to a thickness of 130 g/m2. The coated strip is then annealed.

Figure 2 shows a three-point bending test to measure the bendability. The bending angle is shown on the vertical axis, indicated with A. In the figure tests with prior art zinc coated steel sheet are shown as column PA (prior art), and tests with the zinc coated steel sheet according to the present invention are shown as the column PI (present invention). In this three-point bending test, two rollers with a diameter of 30 mm are disposed at a distance of twice the sheet thickness plus 0.5 mm. The hardened sheet is placed thereon and then subjected to stress with a bending punch having a radius of 0.4 mm at the same distance, respectively, from the rollers. The time, the distance between the contact of the bending punch with the sample and the original position thereof, and the force are measured and recorded. The angle is calculated from the distance. The bending angle at maximum force without cracking on the surface of the specimen is applied as test criterion. It can be seen that for a steel sheet (1.5 mm) of the 22MnB5 type with zinc coated GA130 according to the prior art (PA) a bending angle of about 50° can be reached, whereas with comparable zinc coated steel produced according to the invention (PI), a bending angle of about 75° can be reached. This is a mayor improvement.

## Claims

1. Product formed by hot forming of a metallic coated steel sheet, wherein the formed product has a substrate layer of hot formed steel, a metal affected zone and a diffusion coating layer on the substrate layer, and optionally a metal oxide layer on the diffusion coating layer, the steel having the following composition in weight %:
C: 0.10 - 0.5, preferably 0.15 - 0.4
Mn: 0.5 - 3.0, preferably 1.0 - 2.5
Si: 0.1 - 0.5, preferably 0.1 - 0.4
Cr: up to 1.0, preferably up to 0.8
Ti: up to 0.2, preferably up to 0.1
Al: up to 0.2, preferably up to 0.1
P: up to 0.1, preferably up to 0.08
S: up to 0.05, preferably up to 0.04
B: 0.0005 - 0.08, preferably 0.0005 - 0.04
optionally Nb up to 2, preferably up to 0.1
optionally V up to 2, preferably up to 0.1
optionally W up to 3, preferably up to 0.1
the remainder being iron and unavoidable impurities.
**characterised in that** a low carbon zone is present between the substrate layer and the metal affected zone, wherein the metal affected zone has a thickness of less than 10 µm, and wherein the low carbon layer has a thickness of up to 30 µm

2. Product according to claim 1, wherein the metal of the metallic coated steel sheet is zinc or a zinc alloy, or aluminium or an aluminium alloy.

3. Product according to claim 1 or 2, wherein the low carbon zone has a carbon content of at most 0.01 weight% C.

4. Product according to any one of the preceding claims, wherein the metal affected zone has a thickness of less than 5 µm.

5. Product according to any one of the preceding claims, wherein the low carbon layer has a thickness between 5 and 30 µm, more preferably between 5 and 20 µm, most preferably between 5 and 10 µm.

6. Product according to any one of the preceding claims, wherein the metal of the metallic coated steel sheet is galvannealed zinc, or a zinc alloy containing (in weight%) 0.1 - 6 Al, 0 - 6 Mg and optionally at most 0.2 weight% of Pb, Sb, Ti, Ca, Mn, Sn, La, Ce, Cr, Ni, Zr and/or Bi each, the remainder being zinc and unavoidable impurities, and preferably 0.1 - 3 Al, 0 - 3 Mg and at most 0.2 weight% of Pb, Sb, Ti, Ca, Mn, Sn, La, Ce, Cr, Ni, Zr and/or Bi each, the remainder being zinc and unavoidable impurities, or wherein the metal of the metallic coated steel sheet is a zinc-nickel alloy containing (in weight%) 0.2 - 7 Ni, the remainder being zinc and unavoidable impurities, or wherein the metal of the metallic coated steel sheet is an aluminium alloy containing (in weight%) 6 - 12 Al and/or 1 - 5 Fe, the remainder being aluminium and unavoidable impurities.

7. Method for producing a metallic coated hot formed product, the method comprising the following steps:
- providing a strip of hot formable steel having the following composition in weight %:
C: 0.10 - 0.5, preferably 0.15 - 0.4
Mn: 0.5 - 3.0, preferably 1.0 - 2.5
Si: 0.1 - 0.5, preferably 0.1 - 0.4
Cr: up to 1.0, preferably up to 0.8
Ti: up to 0.2, preferably up to 0.1
Al: up to 0.2, preferably up to 0.1
P: up to 0.1, preferably up to 0.08
S: up to 0.05, preferably up to 0.04
B: 0.0005 - 0.08, preferably 0.0005 - 0.04
optionally Nb up to 2, preferably up to 0.1
optionally V up to 2, preferably up to 0.1
optionally W up to 3, preferably up to 0.1
the remainder being iron and unavoidable impurities;
- annealing said strip by applying a dew point in the range of -15°C to +5°C in an (N2 + H2) atmosphere at 740 to 860 °C for 30 - 240 seconds so that said strip has a decarburized zone with a controlled depth at both sides of it;
- providing a metallic coating on the decarburized steel strip;
- cutting a blank from the coated strip of metal;
- hot forming the coated blank or preformed part into a metallic coated hot formed product.

8. Method for producing a metallic coated hot formed product, the method comprising the following steps:
- hot rolling a hot formable steel having the following composition in weight %:
C: 0.10 - 0.5, preferably 0.15 - 0.4
Mn: 0.5 - 3.0, preferably 1.0 - 2.5
Si: 0.1 - 0.5, preferably 0.1 - 0.4
Cr: up to 1.0, preferably up to 0.8
Ti: up to 0.2, preferably up to 0.1
Al: up to 0.2, preferably up to 0.1
P: up to 0.1, preferably up to 0.08
S: up to 0.05, preferably up to 0.04
B: 0.0005 - 0.08, preferably 0.0005 - 0.04
optionally Nb up to 2, preferably up to 0.1
optionally V up to 2, preferably up to 0.1
optionally W up to 3, preferably up to 0.1
the remainder being iron and unavoidable impurities,
from a finishing rolling temperature between the Ac1 and the Ac3 temperature to the coiling temperature between 450 °C and 750 °C to provide a strip of hot formable steel having a decarburized zone with a controlled depth at both sides of the strip of steel;
- cutting a blank from the coated strip of metal;
- hot forming the coated blank or preformed part into a metallic coated hot formed product.

9. Method according to claim 7 or 8, wherein the hot forming is performed by either heating the blank, hot pressing the blank into a formed product, and quenching the formed product, or cold pressing the blank into a preformed product, heating the preformed product, hot pressing the preformed product into a formed product, and quenching the formed product.

10. Method according to claim 7 to 9, wherein the decarburized zone has been provided to a depth of 20 to 50 µm, preferably a depth of 35 to 45 µm, more preferably a depth of 30 to 40 µm.

11. Method according to any one of claims 7 - 10, wherein the metallic coating on the steel strip is provided as a zinc or zinc alloy, or aluminium or aluminium alloy coating, preferably by using hot-dip coating.

## Patentansprüche

1. Produkt, das durch Warmumformen eines metallbeschichteten Stahlblechs umgeformt wird, wobei das umgeformte Produkt eine Substratschicht aus warmumgeformtem Stahl, eine durch Metall beeinflusste Zone und eine Diffusionsbeschichtungsschicht auf der Substratschicht und optional eine Metalloxidschicht auf der Diffusionsbeschichtungsschicht aufweist, wobei der Stahl folgende Zusammensetzung in Gew.-% aufweist:
C: 0,10 - 0,5, vorzugsweise 0,15 - 0,4
Mn: 0,5 - 3,0, vorzugsweise 1,0 - 2,5
Si: 0,1 - 0,5, vorzugsweise 0,1 - 0,4
Cr: bis zu 1,0, vorzugsweise bis zu 0,8
Ti: bis zu 0,2, vorzugsweise bis zu 0,1
Al: bis zu 0,2, vorzugsweise bis zu 0,1
P: bis zu 0,1, vorzugsweise bis zu 0,08
S: bis zu 0,05, vorzugsweise bis zu 0,04
B: 0,0005 - 0,08, vorzugsweise 0,0005 - 0,04
optional Nb bis zu 2, vorzugsweise bis zu 0,1
optional V bis zu 2, vorzugsweise bis zu 0,1
optional W bis zu 3, vorzugsweise bis zu 0,1
wobei es sich bei dem Rest um Eisen und unvermeidbare Verunreinigungen handelt,
**dadurch gekennzeichnet, dass** zwischen der Substratschicht und der durch Metall beeinflussten Zone eine kohlenstoffarme Zone vorhanden ist, wobei die durch Metall beeinflusste Zone eine Dicke von weniger als 10 µm aufweist und wobei die kohlenstoffarme Schicht eine Dicke von bis zu 30 µm aufweist.

2. Produkt nach Anspruch 1, wobei das Metall des metallbeschichteten Stahlblechs Zink oder eine Zinklegierung oder Aluminium oder eine Aluminiumlegierung ist.

3. Produkt nach Anspruch 1 oder 2, wobei die kohlenstoffarme Zone einen Kohlenstoffgehalt von höchstens 0,01 Gew.-% C aufweist.

4. Produkt nach einem der vorhergehenden Ansprüche, wobei die durch Metall beeinflusste Zone eine Dicke von weniger als 5 µm aufweist.

5. Produkt nach einem der vorhergehenden Ansprüche, wobei die kohlenstoffarme Schicht eine Dicke zwischen 5 und 30 µm, besonders bevorzugt zwischen 5 und 20 µm, am meisten bevorzugt zwischen 5 und 10 µm aufweist.

6. Produkt nach einem der vorhergehenden Ansprüche, wobei das Metall des metallbeschichteten Stahlblechs galvannealed Zink oder eine Zinklegierung ist, die (in Gew.-%) 0,1 - 6 Al, 0 - 6 Mg und optional jeweils höchstens 0,2 Gew.-% Pb, Sb, Ti, Ca, Mn, Sn, La, Ce, Cr, Ni, Zr und/oder Bi, wobei es sich beim Rest um Zink und unvermeidbare Verunreinigungen handelt, und vorzugsweise 0,1 bis 3 Al, 0 bis 3 Mg und jeweils höchstens 0,2 Gew.-% Pb, Sb, Ti, Ca, Mn, Sn, La, Ce, Cr, Ni, Zr und/oder Bi, wobei es sich beim Rest um Zink und unvermeidbare Verunreinigungen handelt, enthält, oder wobei das Metall des metallbeschichteten Stahlblechs eine Zink-Nickel-Legierung ist, die (in Gew.-%) 0,2 bis 7 Ni enthält, wobei es sich beim Rest um Zink und unvermeidbare Verunreinigungen handelt, oder wobei das Metall des metallbeschichteten Stahlblechs eine Aluminiumlegierung ist, die (in Gew.-%) 6 bis 12 Al und/oder 1 - 5 Fe, wobei es sich beim Rest um Aluminium und unvermeidbare Verunreinigungen handelt, enthält.

7. Verfahren zur Herstellung eines metallbeschichteten warmumgeformten Produkts, wobei das Verfahren folgende Schritte umfasst:
Bereitstellen eines Bandes aus warmumformbarem Stahl, der folgenden Zusammensetzung in Gew.-% aufweist:
C: 0,10 - 0,5, vorzugsweise 0,15 - 0,4
Mn: 0,5 - 3,0, vorzugsweise 1,0 - 2,5
Si: 0,1 - 0,5, vorzugsweise 0,1 - 0,4
Cr: bis zu 1,0, vorzugsweise bis zu 0,8
Ti: bis zu 0,2, vorzugsweise bis zu 0,1
Al: bis zu 0,2, vorzugsweise bis zu 0,1
P: bis zu 0,1, vorzugsweise bis zu 0,08
S: bis zu 0,05, vorzugsweise bis zu 0,04
B: 0,0005 - 0,08, vorzugsweise 0,0005 - 0,04
optional Nb bis zu 2, vorzugsweise bis zu 0,1
optional V bis zu 2, vorzugsweise bis zu 0,1
optional W bis zu 3, vorzugsweise bis zu 0,1, wobei es sich beim Rest um Eisen und unvermeidbare Verunreinigungen handelt; Glühen des Bandes durch Anlegen eines Taupunkts im Bereich von -15 °C bis + 5 °C in einer (N2 + H2)-Atmosphäre bei 740 bis 860 °C 30 bis 240 Sekunden lang, so dass das Band eine entkohlte Zone mit einer kontrollierten Tiefe auf seinen beiden Seiten aufweist;
- Bereitstellen einer Metallbeschichtung auf dem entkohlten Stahlband;
- Schneiden eines Rohlings aus dem beschichteten Metallband;
- Warmumformen des beschichteten Rohlings oder vorumgeformten Teils zu einem metallbeschichteten warmumgeformten Produkt.

8. Verfahren zur Herstellung eines metallbeschichteten warmumgeformten Produkts, wobei das Verfahren folgende Schritte umfasst:
Warmwalzen eines warmumformbaren Stahls, der folgende Zusammensetzung in Gew.-% aufweist:
C: 0,10 - 0,5, vorzugsweise 0,15 - 0,4
Mn: 0,5 - 3,0, vorzugsweise 1,0 - 2,5
Si: 0,1 - 0,5, vorzugsweise 0,1 - 0,4
Cr: bis zu 1,0, vorzugsweise bis zu 0,8
Ti: bis zu 0,2, vorzugsweise bis zu 0,1
Al: bis zu 0,2, vorzugsweise bis zu 0,1
P: bis zu 0,1, vorzugsweise bis zu 0,08
S: bis zu 0,05, vorzugsweise bis zu 0,04
B: 0,0005 - 0,08, vorzugsweise 0,0005 - 0,04
optional Nb bis zu 2, vorzugsweise bis zu 0,1
optional V bis zu 2, vorzugsweise bis zu 0,1
optional W bis zu 3, vorzugsweise bis zu 0,1
wobei es sich beim Rest um Eisen und unvermeidbare Verunreinigungen handelt, von einer Fertigwalztemperatur zwischen der Acl- und der Ac3-Temperatur bis zur Wickeltemperatur zwischen 450 °C und 750 °C, um ein Band aus warmumformbarem Stahl bereitzustellen, das eine entkohlte Zone mit einer kontrollierten Tiefe an beiden Seiten des Stahlbands aufweist;
- Schneiden eines Rohlings aus dem beschichteten Metallband;
- Warmumformen des beschichteten Rohlings oder vorumgeformten Teils zu einem metallbeschichteten warmumgeformten Produkt.

9. Verfahren nach Anspruch 7 oder 8, wobei das Warmumformen entweder durch Erwärmen des Rohlings, Warmpressen des Rohlings zu einem umgeformten Produkt und Abschrecken des umgeformten Produkts oder Kaltpressen des Rohlings zu einem vorumgeformten Produkt, Erwärmen des vorumgeformten Produkts, Warmpressen des vorumgeformten Produkts zu einem umgeformten Produkt und Abschrecken des umgeformten Produkts durchgeführt wird.

10. Verfahren nach Anspruch 7 bis 9, wobei die entkohlte Zone bis zu einer Tiefe von 20 bis 50 µm, vorzugsweise einer Tiefe von 35 bis 45 µm, besonders bevorzugt einer Tiefe von 30 bis 40 µm bereitgestellt worden ist.

11. Verfahren nach einem der Ansprüche 7 bis 10, wobei die Metallbeschichtung auf dem Stahlband als Zink- oder Zinklegierungs- oder Aluminium- oder Aluminiumlegierungsbeschichtung bereitgestellt wird, vorzugsweise unter Verwendung einer Schmelztauchbeschichtung.

## Revendications

1. Produit mis en forme par formage à chaud d'une tôle d'acier métallisée, le produit mis en forme possédant une couche de substrat en acier mis en forme à chaud, une zone affectée par le métal et une couche de revêtement par diffusion sur la couche de substrat, et éventuellement une couche d'oxyde métallique sur la couche de revêtement par diffusion, l'acier possédant la composition suivante exprimée en % en poids :
C : 0,10-0,5, de préférence 0,15-0,4
Mn : 0,5-3,0, de préférence 1,0-2,5
Si : 0,1-0,5, de préférence 0,1-0,4
Cr : jusqu'à 1,0, de préférence jusqu'à 0,8
Ti : jusqu'à 0,2, de préférence jusqu'à 0,1
Al : jusqu'à 0,2, de préférence jusqu'à 0,1
P : jusqu'à 0,1, de préférence jusqu'à 0,08
S : jusqu'à 0,05, de préférence jusqu'à 0,04
B : 0,0005-0,08, de préférence 0,0005-0,04
éventuellement Nb jusqu'à 2, de préférence jusqu'à 0,1
éventuellement V jusqu'à 2, de préférence jusqu'à 0,1
éventuellement W jusqu'à 3, de préférence jusqu'à 0,1
le reste étant du fer et des impuretés inévitables,
**caractérisé en ce qu'**une zone à faible teneur en carbone est présente entre la couche de substrat et la zone affectée par le métal, ladite zone affectée par le métal possédant une épaisseur inférieure à 10 µm, et ladite couche à faible teneur en carbone possédant une épaisseur allant jusqu'à 30 µm.

2. Produit selon la revendication 1, ledit métal de la tôle d'acier métallisée étant du zinc ou un alliage de zinc, ou de l'aluminium ou un alliage d'aluminium.

3. Produit selon la revendication 1 ou 2, ladite zone à faible teneur en carbone possédant une teneur en carbone inférieure ou égale à 0,01 % en poids de C.

4. Produit selon l'une quelconque des revendications précédentes, ladite zone affectée par le métal possédant une épaisseur inférieure à 5 µm.

5. Produit selon l'une quelconque des revendications précédentes, ladite couche à faible teneur en carbone possédant une épaisseur comprise entre 5 et 30 µm, de préférence entre 5 et 20 µm, idéalement entre 5 et 10 µm.

6. Produit selon l'une quelconque des revendications précédentes, ledit métal de la tôle d'acier métallisée étant du zinc recuit après galvanisation de zinc ou un alliage de zinc contenant (en % en poids) 0,1-6 d'Al, 0-6 de Mg et éventuellement au plus 0,2 % en poids de Pb, Sb, Ti, Ca, Mn, Sn, La, Ce, Cr, Ni, Zr et/ou Bi chacun, le reste étant du zinc et des impuretés inévitables, et de préférence 0,1-3 d'Al, 0-3 de Mg et au plus 0,2 % en poids de Pb, Sb, Ti, Ca, Mn, Sn, La, Ce, Cr, Ni, Zr et/ou Bi chacun, le reste étant du zinc et des impuretés inévitables, ou ledit métal de la tôle d'acier métallisée étant un alliage de zinc-nickel contenant (en % en poids) 0,2-7 de Ni, le reste étant du zinc et des impuretés inévitables, ou ledit métal de la tôle d'acier métallisée étant un alliage d'aluminium contenant (en % en poids) 6-12 d'Al et/ou 1-5 de Fe, le reste étant de l'aluminium et des impuretés inévitables.

7. Procédé permettant la production d'un produit mis en forme à chaud métallisé, le procédé comprenant les étapes suivantes :
- fourniture d'une bande d'acier pouvant être mis en forme à chaud possédant la composition suivante exprimée en % en poids :
C : 0,10-0,5, de préférence 0,15-0,4
Mn : 0,5-3,0, de préférence 1,0-2,5
Si : 0,1-0,5, de préférence 0,1-0,4
Cr : jusqu'à 1,0, de préférence jusqu'à 0,8
Ti : jusqu'à 0,2, de préférence jusqu'à 0,1
Al : jusqu'à 0,2, de préférence jusqu'à 0,1
P : jusqu'à 0,1, de préférence jusqu'à 0,08
S : jusqu'à 0,05, de préférence jusqu'à 0,04
B : 0,0005-0,08, de préférence 0,0005-0,04
éventuellement Nb jusqu'à 2, de préférence jusqu'à 0,1
éventuellement V jusqu'à 2, de préférence jusqu'à 0,1
éventuellement W jusqu'à 3, de préférence jusqu'à 0,1
le reste étant du fer et des impuretés inévitables ;
- recuit de ladite bande en appliquant un point de rosée dans la plage allant de -15°C à +5°C dans une atmosphère (N2+H2) à une température allant de 740 à 860°C pendant 30 à 240 secondes afin que ladite bande possède une zone décarburée avec une profondeur régulée sur les deux côtés de celle-ci ;
- fourniture d'un revêtement métallique sur la bande d'acier décarburée ;
- découpe d'une ébauche à partir de la bande de métal revêtue ;
- formage à chaud de l'ébauche revêtue ou de la pièce préformée en un produit mis en forme à chaud métallisé.

8. Procédé permettant la production d'un produit mis en forme à chaud métallisé, le procédé comprenant les étapes suivantes :
- laminage à chaud d'un acier pouvant être mis en forme à chaud possédant la composition suivante exprimée en % en poids :
C : 0,10-0,5, de préférence 0,15-0,4
Mn : 0,5-3,0, de préférence 1,0-2,5
Si : 0,1-0,5, de préférence 0,1-0,4
Cr : jusqu'à 1,0, de préférence jusqu'à 0,8
Ti : jusqu'à 0,2, de préférence jusqu'à 0,1
Al : jusqu'à 0,2, de préférence jusqu'à 0,1
P : jusqu'à 0,1, de préférence jusqu'à 0,08
S : jusqu'à 0,05, de préférence jusqu'à 0,04
B : 0,0005-0,08, de préférence 0,0005-0,04
éventuellement Nb jusqu'à 2, de préférence jusqu'à 0,1
éventuellement V jusqu'à 2, de préférence jusqu'à 0,1
éventuellement W jusqu'à 3, de préférence jusqu'à 0,1
le reste étant du fer et des impuretés inévitables, à partir d'une température de laminage de finition comprise entre les températures Ac1 et Ac3 jusqu'à la température de bobinage comprise entre 450°C et 750°C pour fournir une bande d'acier pouvant être mis en forme à chaud possédant une zone décarburée avec une profondeur régulée sur les deux côtés de la bande d'acier ;
- découpe d'une ébauche de la bande de métal revêtue ;
- formage à chaud de l'ébauche revêtue ou de la pièce préformée en un produit mis en forme à chaud métallisé.

9. Procédé selon la revendication 7 ou 8, ledit formage à chaud étant effectué soit en chauffant l'ébauche, en pressant à chaud l'ébauche en un produit mis en forme, et en effectuant la trempe du produit mis en forme, soit en pressant à froid l'ébauche en un produit préformé, en chauffant le produit préformé, en pressant à chaud le produit préformé en un produit mis en forme et en effectuant la trempe du produit mis en forme.

10. Procédé selon les revendications 7 à 9, ladite zone décarburée ayant été disposée à une profondeur de 20 à 50 µm, de préférence une profondeur de 35 à 45 µm, idéalement à une profondeur de 30 à 40 µm.

11. Procédé selon l'une quelconque des revendications 7 à 10, ledit revêtement métallique sur la bande d'acier étant fourni sous forme de zinc ou d'alliage de zinc, ou de revêtement d'aluminium ou d'alliage d'aluminium, de préférence à l'aide d'un revêtement par immersion à chaud.
